

# UNITED STATES PATENT OFFICE.

FREDERICK M. BECKET, OF NIAGARA FALLS, NEW YORK, ASSIGNOR TO  
ELECTRO METALLURGICAL COMPANY, A CORPORATION OF WEST  
VIRGINIA.

## METHOD OF TREATING IRON OR STEEL.

No. 858,326.

Specification of Letters Patent.

Patented June 25, 1907.

Application filed March 13, 1907. Serial No. 362,224.

*To all whom it may concern.*

Be it known that I, FREDERICK M. BECKET, a subject of the King of Great Britain, residing at Niagara Falls, in the county of Niagara and State of New York, have invented certain new and useful Improvements in Methods of Treating Iron or Steel, of which the following is a specification.

This invention is a method of treating iron or steel and removing therefrom gaseous and other impurities which exert a deleterious effect on the metal; according to the invention there is incorporated with the molten metal an alloy containing titanium and calcium, preferably but not necessarily associated with aluminium and silicon, carbon being usually present in greater or less proportion in accordance with the method of manufacture employed. Iron is also usually present as a component of the alloy, derived from the ores employed in its manufacture.

It is well known that gases, particularly nitrogen, hydrogen and carbon monoxide, are occluded by molten steel and tend to separate therefrom at the moment of solidification, and it is customary to add to the steel, usually at the time of casting, either aluminium or an alloy containing aluminium, for the purpose of eliminating such gases. In order to effect a commercially complete elimination of such gases and also the further result of a substantial reduction of the percentage of sulfur and dissolved metallic oxides, and to some extent the reduction of the percentage of phosphorus, I propose the use, preferably in the manner above indicated and in proportions dependent upon the kind of iron or steel and the percentage of impurities therein, of the alloy containing titanium and calcium above referred to.

I may produce an alloy containing titanium and calcium by reduction by carbon in an electric furnace of a charge containing oxides or oxygen compounds of titanium and calcium, usually with the addition of silica in proportion depending upon the percentage of silicon desired. The reduction of the mixed oxides yields a product of metallic character instead of the carbid which would result from the reduction of either oxid alone. In addition to its value as an ingredient of the alloy for use in the treatment of iron or steel, silicon acts to a marked degree to diminish the percentage of carbon in the

product; this is of advantage for the reason that a product low in carbon can be added, if desired, in relatively large proportions to iron or steel without unduly increasing the proportion of carbon in the resulting metal.

When an alloy containing aluminium in addition to titanium and calcium is desired, it is most conveniently produced by reduction in an electric furnace having an electrode or electrodes of carbon, of a charge containing oxides of titanium and calcium, or of titanium, calcium and silicon, by means of metallic aluminium used in proportion to yield an aluminium-bearing alloy; or a mixture of the oxides of titanium, calcium and aluminium, or of titanium, calcium, aluminium and silicon, may be reduced by carbon. In any case the operation is preferably rendered continuous in character by adding fresh portions of the charge from time to time, and tapping the molten alloy as desired.

An example of the composition of alloys I have produced for the purpose indicated is shown by the following analysis:

|           |       |           |    |
|-----------|-------|-----------|----|
| Titanium  | 50.67 | per cent. | 80 |
| Calcium   | 8.32  | "         |    |
| Aluminium | 22.50 | "         |    |
| Iron      | 11.83 | "         |    |
| Silicon   | 4.20  | "         | 85 |
| Carbon    | 1.86  | "         |    |
| Total     | 99.38 |           |    |

It will be understood that the proportions of the several components of the alloy, or the presence therein of aluminium or silicon, is determined by the composition of the charge smelted. The alloy is varied in composition according to the percentage of one or more of its constituents desired in the finished iron or steel, and also according to the particular class of iron or steel to be treated.

The appearance of the alloy varies in accordance with its composition, mode and scale of production, rate of cooling, etc.: in general it exists as a light gray or grayish product of metallic appearance but without pronounced luster or distinct crystalline structure, of moderate hardness. Particularly when a considerable proportion of calcium is present it is subject to slow decomposition in water or moist air.

It is not practicable to state with certainty

the complete function of each ingredient of the above described alloy. It may be assumed, however, that the titanium acts chiefly upon the occluded nitrogen; the calcium upon the nitrogen, hydrogen, sulfur, the dissolved oxids, and to some extent phosphorus; the aluminium upon the carbon monoxid and dissolved oxids; and the silicon upon the hydrogen and dissolved oxids. This assumption is based upon the observed facts that alloys of this type exert a beneficial action upon steel and reduce the proportion of impurities therein, taken in connection with the fact that the constituent elements of the alloys are known to form stable compounds with the elements which they are assumed to remove. The result of the addition of the combined elements is to eliminate a very substantial proportion of the impurities commonly existing in iron or steel. As compared with ferrotitanium the alloy possesses a relatively low melting point, and is much more readily incorporated with the molten metal and distributed therethrough.

25 I claim:

1. The method of treating iron or steel

which consists in incorporating with the molten metal an alloy containing titanium and calcium.

2. The method of treating iron or steel which consists in incorporating with the molten metal an alloy containing titanium, calcium and aluminium.

3. The method of treating iron or steel which consists in incorporating with the molten metal an alloy containing titanium, calcium, aluminium and silicon.

4. The method of treating iron or steel which consists in incorporating with the molten metal an alloy containing titanium, calcium, aluminium, silicon, and carbon.

5. The method of treating iron or steel which consists in incorporating with the molten metal an alloy containing titanium, calcium, aluminium, silicon, carbon, and iron.

In testimony whereof, I affix my signature in presence of two witnesses.

FREDERICK M. BECKET.

Witnesses:

C. C. MOSHER,  
J. N. DEINHARDT.